

Dec. 23, 1958

W. F. SCHROEDER  
PROCESS OF BLEACHING KRAFT PULP WITH ALKALINE HYPOCHLORITE  
BLEACH ACIDIFYING THE PULP CONTAINING RESIDUAL CHLORINE  
AND THEN BLEACHING WITH ALKALINE PEROXIDE  
Filed Dec. 7, 1953



WILLARD F. SCHROEDER  
INVENTOR.

BY *E. J. Berry*

ATTORNEY

1

2,865,701

**PROCESS OF BLEACHING KRAFT PULP WITH  
ALKALINE HYPOCHLORITE BLEACH ACIDIFY-  
ING THE PULP CONTAINING RESIDUAL CHLO-  
RINE AND THEN BLEACHING WITH ALKALINE  
PEROXIDE**

Willard F. Schroeder, Ashtabula, Ohio, assignor to National Distillers and Chemical Corporation, a corporation of Virginia

Application December 7, 1953, Serial No. 396,709

2 Claims. (Cl. 8—106)

This invention is concerned with a new process for bleaching of wood pulp which produces a surprising and unexpected bleach response using a preoxide treatment in the last bleaching stage. This new technique is based on a combination of stages employing critical factors and is readily adaptable to and/or incorporated into existing multi-stage bleaching operations. The process yields bleached pulps having both superior brightness stability and strength properties.

Although it has previously been shown that the use of a peroxide bleach in the last stage of kraft pulp bleaching produced a more brightness-stable pulp than any other bleaching agent, the bleach response of the pulp to peroxide in the last stage was found to be quite poor compared with hypochlorite or chlorine dioxide. Various methods have been proposed to solve this problem. For example, the use of sodium peroxide in the last alkaline extraction stage has been suggested as a means of improving the final pulp brightness but the brightness stability of the pulp was found to be inferior. Also, the superbleaching of kraft wood pulp with peroxide at high consistency for relatively long time periods has also been advocated as a means of improving bleach response. Because of the lower alkalinity of the formula in this procedure, the brightness stability is not as good as that of the process herein described. However, this technique requires a large storage area for the bleaching pulp and expenditures for additional equipment and results in high labor cost and inflexibility of operation.

A very satisfactory method has been found for improving the bleach response of peroxide and, more particularly, of sodium peroxide in the last bleaching stage where peroxide can be used to the best advantage. This results in a better final brightness of the pulp and also in a better brightness stability of the bleached pulp. The final pulp strength is also high if proper critical factors are satisfactorily controlled.

In using this novel technique in a typical four or five stage process, the unbleached kraft pulp is first chlorinated and alkaline extracted in the usual manner, or any other known initial sequence of steps can be employed. Following these preliminary steps, a hydrochlorite bleaching stage is carried out. The alkalinity of the hypochlorite bleach is adjusted at a high level to give a pH value of about  $9.5 \pm 1.0$  pH units in about one-half to two-thirds the normal bleaching time for the alkaline hypochlorite stage, e. g. one to two hours bleaching time rather than  $1\frac{1}{2}$  to 3 hours. The residual chlorine remaining on the pulp should be between 10% and 35%, based on the total amount added. The pulp is preferably then diluted to 3% to 6% consistency and adjusted to a pH of about 5 with a mineral acid, preferably sulfuric acid or hydrochloric acid. After a period of from one to thirty minutes, the pulp is then washed in a normal manner and

2

given at least one final stage bleach using 0.1 to 1.0% sodium peroxide at above  $120^{\circ}$  F., preferably  $140^{\circ}$  to  $160^{\circ}$  F., the pulp having 12% to 16% consistency. It has been found that the final peroxide bleach stage can also be quite satisfactorily carried out on a pulp having a density of less than 10%, for example, 4 to 8%. When the above-described combination and sequence of steps is used, the final pulp brightness is much higher than when this method is not used, and the pulp has a higher cupri-  
10 ethylenediamine disperse viscosity. The use of this improved technique further results in a brighter pulp having equivalent brightness stability than does an alkaline extraction followed by a bleach in the normal manner with hypochlorite, washing, an alkaline extraction, and an identical last stage sodium peroxide bleach. For the best final results, there should be maximum pulp brightness combined with maximum pulp strength.

The sequence or combination of steps involved in the practice of the invention shows the striking results when applied to chemical wood pulp especially prepared by an alkaline pulping process such as kraft or soda pulp, although the method can, if desired, also be applied to sulfite pulp. It is not considered suitable for use on the mechanical type pulps since this pulp type is not normally bleached with a multi-stage process, but rather a single stage process is used. The large amount of hypochlorite required to give the above-described effect prior to a peroxide bleach would make the process uneconomical when used on mechanical type pulp.  
20 In preliminary preparation of pulp, the customary bleaching operations may be used without significant changes in procedure. In general, the initial bleaching is some type of chlorine treatment. This step may be either a straight chlorine treatment or it may be carried out by first adding chlorine followed by the addition of lime after a few minutes. The next step, in either case, will be an alkaline extraction stage using normal conditions as practiced in the pulp industry. Thus, the pulp is in condition for the sequence of steps which gives the outstanding brightness and pulp strength qualities which are characteristic of this improvement.

The next stage or treatment step, characterized in the examples as the third stage, constitutes a hypochlorite treatment. In this stage, an alkaline hypochlorite is used, and both sodium and calcium hypochlorite have been found quite satisfactory. To achieve best results, this hypochlorite treatment is carried out so that approximately 65 to 90% of the available chlorine is consumed. Or, stated another way, there should be about 10 to 35% residual chlorine remaining based on the amount originally added. Compared to the usual conditions of operation, in order to accomplish this, there should be either a higher level of alkalinity used and/or the bleach period should be limited to a shorter period of time. The latter procedure is preferable. The pH of the pulp at the end of this step should be about  $9.5 \pm 1.0$  pH units. Thus, if the hypochlorite stage is too long or is carried out under conditions which are too drastic, the final brightness may be very good but the pulp strength will be lowered considerably. Thus, if the residual chlorine falls below 10%, the hypochlorite stage has been of too long duration and the final pulp strength will be undesirably low.

If the residual chlorine is too high (above about 35%), this indicates that the hypochlorite treatment has not been strenuous enough to accomplish the necessary bleaching action and thereby give the pulp the required brightness.

It is recommended that the hypochlorite bleaching time with this technique be about one-half to two-thirds of

that normally used which is approximately 1½ to 3 hours.

The acid treatment which is an integral part of this invention is best characterized, not as a separate step, but rather as an additional or supplemental part of the hypochlorite treatment. In carrying out studies to establish the best sequence of treating steps, it has been found best not to wash the pulp after the hypochlorite bleaching treatment. In other words, rather than washing the pulp following the hypochlorite treatment, better pulp brightness results are obtained if it is directly and immediately thereafter treated with acid under controlled conditions.

In carrying out the acid treating stage, a number of critical factors should be carefully controlled in order to obtain the best results. The acid used should be of the mineral type and is preferably non-reducing. Thus, either sulfuric acid or hydrochloric acid can be used quite satisfactorily but,  $\text{SO}_2$ , a reducing acid, has been found to give less satisfactory results. Also, alum, a commonly employed acidifying agent, does not give good results.

The pH of the pulp should be adjusted to a value of approximately 5. A slight variation in pH of from about 4 up to 5.5 can be allowed. If a pH of 6 is used, much poorer results are obtained, and pH values of less than 4 also give mediocre improvement. This variable is very critical and should be carefully controlled in order to achieve the outstanding results of the invention.

With regard to the time of treatment, this is dependent somewhat upon the nature of the various commercial pulp bleaching systems. However, it has been observed that prolonged acid treatments are little more effective than relatively shorter periods of from 1 up to 15 minutes.

Although it is not believed to constitute a critical factor in the treatment, it has also been observed that the results given by acid treating a high density pulp of 12 to 16% consistency are somewhat better than those obtained from treating a lower density pulp of 3 to 6%. However, superior brightness values are obtained in either case and it is not intended to limit the invention to pulp having any particular densities. This is an advantage since it avoids the necessity of thickening or diluting the pulp prior to using the acid treatment.

The effect of the temperature during the acid treatment has been found not to be critical. A temperature within the range of 35 to 100° F. can be employed.

Most important to the ultimate success of the invention is the carrying out of the hypochlorite bleach such that there is a relatively high residual available chlorine. It is only in this way that there is obtained a better response in the final peroxide bleach stage.

Following the acid treatment at least one peroxide bleaching treatment is used. It is much preferred to use an alkaline peroxide bleach as the final treatment. The alkaline peroxide solution may be prepared from hydrogen peroxide and substantially any fixed alkali or from the alkaline peroxides such as alkali metal peroxides, alkaline earth peroxides, as well as perborates and the like.

This treatment gives improved brightness and brightness stability. A hypochlorite bleach at this stage has been found not as satisfactory. The initial pH in this stage is about  $11 \pm .5$  pH units. The required amount of sodium peroxide ranges from 0.1 up to 1%. The peroxide solution also generally contains 1 to 3% sodium silicate as a buffer and 0.01 to 0.05% Epsom salts as a stabilizer. The alkaline peroxide bleaching treatment can be carried out at 110 to 180° F., and preferably from 140 to 160° F. The consistency preferred for this step is 10 to 20% but low densities of less than 10% consistency also give good results in the peroxide treatment.

In addition, it has been found useful to carry out this final peroxide bleach in more than one stage. Thus, data shows that if the peroxide used in one bleaching stage

is split into two or more separate bleaching stages, the brightness results are equivalent to or better than those obtained in the single stage operation.

The final peroxide bleach improves the brightness stability quite markedly. The acidification step has been shown not to adversely influence the viscosity, pulp polymerization reactions, or pulp strength.

It is to be understood that the herein described sequence of steps can be used in conjunction with any pulp process wherein chemical pulp is subjected to multiple bleaching operations. It can be incorporated into the process either subsequent to or prior to other stages for bleaching and other treatments.

The invention will be further illustrated by the following examples. The brightness values shown are measured on a percent reflectance scale in which magnesium oxide is taken as 100%. The brightness values shown were measured on a Hunter reflectometer. The density or consistency is measured on the basis of oven dry pulp weight. The percent residual chlorine values are based on the amount of residual chlorine at the end of the hypochlorite bleach.

The kraft wood pulps used in Examples I through IX below were subjected to various preliminary bleaching stages, each series of which differed slightly. These different kraft pulp samples will be identified in the following examples as pulps A and B. The individual stage treatments of these pulps are shown in the following outline:

|    | Pulp | Wood Species  | Stage I                | Stage II         |
|----|------|---------------|------------------------|------------------|
| 35 | A    | Southern Pine | 5.0% Av. $\text{Cl}_2$ | 2.0% NaOH.       |
|    |      |               | 3.5% Consistency       | 13% Consistency. |
| 40 | B    | Douglas Fir   | 55-70° F.              | 100° F.          |
|    |      |               | pH 1.5-1.9             | pH 11+           |
|    |      |               | 45 minutes             | 2 hours.         |
|    |      |               | 4.5% Av. $\text{Cl}_2$ | 2.4% NaOH.       |
|    |      |               | 3.5% Consistency       | 16% Consistency. |
|    |      |               | 55-70° F.              | 100° F.          |
|    |      |               | pH 1.5-1.9             | pH 11+           |
|    |      |               | 1 hour                 | 1½ hours.        |

#### EXAMPLE I

A series of tests was carried out to demonstrate the effectiveness of the invention when the preferred combination of stages is employed in the appropriate sequence. In these experiments pulp Sample A described above was used. In no case was the pulp washed between the hypochlorite treatment and the acid treatment. For the acid treatment stage, the samples were treated at 4% consistency with  $\text{H}_2\text{SO}_4$  to give the final pH shown. The time of the acid treatment stage was approximately 15 minutes and the pulp was washed after the acid treatment, prior to the final peroxide bleach stage. The data obtained is shown in Table 1. From this data it can readily be seen that a higher brightness value is reached and a greater brightness increment is shown for samples having the acid treatment followed by a peroxide bleach. Neither of these steps employed independently, however, gives satisfactory brightness values.

The accompanying figure is a graph of the values of Table 1. This figure clearly summarizes the final outstanding results achieved by the invention. The brightness of the pulp is plotted according to the sequence of stages as shown in Table 1. Each of the three pulp samples was subjected to different hypochlorite bleach periods giving between 10 and 35% chlorine residual values and pH values of  $9.5 \pm 1.0$  pH units. A control pulp which received no acid treatment is also shown. It should be noted that within the preferred chlorine residual values and pH range for the pulp, the final high level of brightness reached after acid treatment and subsequent peroxide treatment is substantially constant. This level is well above the brightness reached by the 75 control sample which received no acid treatment.

Table 1

| Calcium Hypochlorite Bleach Stage      |                   |          |                           | Acid Treatment |         | Na <sub>2</sub> O <sub>2</sub> Bleach  |                                                 | Hunter Brightness of Pulp | Brightness Increment of Bleach |
|----------------------------------------|-------------------|----------|---------------------------|----------------|---------|----------------------------------------|-------------------------------------------------|---------------------------|--------------------------------|
| Percent Available Cl <sub>2</sub> Used | Bleach Time (hr.) | Final pH | Percent Residual Chlorine | Acid used      | Pulp pH | Percent Na <sub>2</sub> O <sub>2</sub> | Percent Residual Na <sub>2</sub> O <sub>2</sub> |                           |                                |
| 2.7                                    | 1                 | 10.35    | 34.9                      | No             |         |                                        |                                                 | 70.5                      |                                |
| 2.7                                    | 1                 | 10.35    | 34.9                      | Yes            | 4.5     |                                        |                                                 | 76.0                      |                                |
| 2.7                                    | 1                 | 10.35    | 34.9                      | Yes            | 4.5     | 0.5                                    | 11.9                                            | 83.6                      | 13.1                           |
| 2.7                                    | 1.5               | 9.6      | 28.8                      | No             |         |                                        |                                                 | 73.4                      |                                |
| 2.7                                    | 1.5               | 9.6      | 28.8                      | Yes            | 4.65    |                                        |                                                 | 77.3                      |                                |
| 2.7                                    | 1.5               | 9.6      | 28.8                      | Yes            | 4.65    | 0.5                                    | 17.3                                            | 84.2                      | 10.8                           |
| 2.7                                    | 2.0               | 8.85     | 21.1                      | No             |         |                                        |                                                 | 75.6                      |                                |
| 2.7                                    | 2.0               | 8.85     | 21.1                      | No             |         | 0.5                                    | 1.1                                             | 78.4                      | 2.8                            |
| 2.7                                    | 2.0               | 8.85     | 21.1                      | Yes            | 4.70    |                                        |                                                 | 79.3                      |                                |
| 2.7                                    | 2.0               | 8.85     | 21.1                      | Yes            | 4.70    | 0.5                                    | 15.1                                            | 84.2                      | 7.6                            |

## EXAMPLE II

A similar, related series of experiments was carried out to study the effects of available chlorine residual and pulp alkalinity on brightness and their relation to pulp viscosities. An alkaline extracted pulp having a viscosity of 19.5 centipoises was used for these tests. The pulp sample A was not washed between the hypochlorite bleaching stage and the acid treatment stage. The data obtained is shown in Table 2 below.

These data show that good final brightness is obtained when the hypochlorite bleaching step is directly followed by an acid treatment and then a peroxide bleach. However, these data show that for any particular sequence, the longer the hypochlorite bleaching stage, the lower the viscosity. Also, if the shorter hypochlorite bleaching period is followed by an acid treatment and then a peroxide bleach, the final pulp brightness is the same as when a longer hypochlorite bleach is used. Thus, the preferred conditions include a relatively shorter hypochlorite bleaching stage followed by acid treatment and peroxide bleaching. Also, the higher the pulp pH and percent residual chlorine of the hypochlorite bleach step,

the higher final viscosity with the equivalent final brightness that is obtained. Therefore, the preferred conditions of the hypochlorite bleach stage yield a pulp having a pH of  $9.5 \pm 1.0$  pH units, and from 10% up to 35% residual chlorine.

## EXAMPLE III

A set of experiments was carried out to determine the effect of various pH values of the acid treatment. A pulp B sample was used for these tests. The calcium hypochlorite bleach stage was the same in each case. The percentage of available chlorine used was 2.0%, and the bleach time was 1.5 hours. Following this treatment, the final pH of the pulp was 8.5, and the residual chlorine value was 18.6%. The pulp samples were not washed prior to the acid treatment stage. The results are shown in Table 3. These data show that the brightness response to the peroxide stage is quite good at a pH of about 5.0. As the pulp becomes less acidic, the brightness response decreases considerably. As the pH approaches 4.0, the brightness response also decreases. A pH value of from 4.0 to 5.5 is preferred and 5.0 appears to give maximum good results.

Table 2

| Calcium Hypochlorite Bleach Stage   |                   |          |                                |                               | Acid Treatment |         | Na <sub>2</sub> O <sub>2</sub> Bleach  |                                               |                               | Hunter Brightness | Brightness Increment of Bleach |
|-------------------------------------|-------------------|----------|--------------------------------|-------------------------------|----------------|---------|----------------------------------------|-----------------------------------------------|-------------------------------|-------------------|--------------------------------|
| Percent Avail. Cl <sub>2</sub> Used | Bleach Time (hr.) | Final pH | Percent Resid. Cl <sub>2</sub> | CED <sup>1</sup> Visc. (cps.) | Acid used      | Pulp pH | Percent Na <sub>2</sub> O <sub>2</sub> | Percent Resid. Na <sub>2</sub> O <sub>2</sub> | CED <sup>1</sup> Visc. (cps.) |                   |                                |
| 2.7                                 | 1.0               | 10.35    | 34.9                           | 10.3                          | No             |         |                                        |                                               |                               | 70.5              |                                |
| 2.7                                 | 1.0               | 10.35    | 34.9                           | -----                         | Yes            | 4.5     |                                        |                                               |                               | 76.0              |                                |
| 2.7                                 | 1.0               | 10.35    | 34.9                           | -----                         | Yes            | 4.5     | 0.5                                    | 11.9                                          | 8.1                           | 83.6              | 13.1                           |
| 2.7                                 | 1.5               | 9.6      | 28.8                           | 9.6                           | No             |         |                                        |                                               |                               | 73.4              |                                |
| 2.7                                 | 1.5               | 9.6      | 28.8                           | -----                         | Yes            | 4.65    |                                        |                                               |                               | 77.3              |                                |
| 2.7                                 | 1.5               | 9.6      | 28.8                           | -----                         | Yes            | 4.65    | 0.5                                    | 17.3                                          | 8.1                           | 84.2              | 10.8                           |
| 2.7                                 | 2.0               | 8.85     | 21.1                           | 9.1                           | No             |         |                                        |                                               |                               | 75.6              |                                |
| 2.7                                 | 2.0               | 8.85     | 21.1                           | 9.1                           | No             |         | 0.5                                    | 1.1                                           | 8.0                           | 78.4              | 2.8                            |
| 2.7                                 | 2.0               | 8.85     | 21.1                           | 9.1                           | Yes            | 4.70    |                                        |                                               |                               | 79.3              |                                |
| 2.7                                 | 2.0               | 8.85     | 21.1                           | 9.1                           | Yes            | 4.70    | 0.5                                    | 15.1                                          | 7.7                           | 84.2              | 7.6                            |
| 2.7                                 | 1.0               | 8.60     | 31.1                           | 10.5                          | No             |         |                                        |                                               |                               | 74.2              |                                |
| 2.7                                 | 1.0               | 8.60     | 31.1                           | -----                         | Yes            | 4.6     |                                        |                                               |                               | 78.8              |                                |
| 2.7                                 | 1.0               | 8.60     | 31.1                           | -----                         | Yes            | 4.6     | 0.5                                    | 21.6                                          | 7.7                           | 83.4              | 9.2                            |
| 2.7                                 | 1.5               | 8.0      | 18.3                           | 9.2                           | No             |         |                                        |                                               |                               | 78.8              |                                |
| 2.7                                 | 1.5               | 8.0      | 18.3                           | -----                         | Yes            | 4.6     |                                        |                                               |                               | 81.0              |                                |
| 2.7                                 | 1.5               | 8.0      | 18.3                           | -----                         | Yes            | 4.6     | 0.5                                    | 15.1                                          | 7.1                           | 84.6              | 6.8                            |
| 2.7                                 | 2.0               | 7.65     | 11.1                           | 8.1                           | No             |         |                                        |                                               |                               | 80.7              |                                |
| 2.7                                 | 2.0               | 7.65     | 11.1                           | -----                         | No             |         | 0.5                                    | 0.4                                           | 6.8                           | 81.3              | 0.6                            |
| 2.7                                 | 2.0               | 7.65     | 11.1                           | 8.1                           | Yes            | 4.9     |                                        |                                               |                               | 81.8              |                                |
| 2.7                                 | 2.0               | 7.65     | 11.1                           | -----                         | Yes            | 4.9     | 0.5                                    | 9.1                                           | 6.5                           | 84.7              | 4.0                            |

<sup>1</sup> TAPPI Standard Method T230sm-50 cupriethylenediamine disperse viscosity for 1/2% pulp solution.

Table 3

| Acid Treatment                 |                     |         |             |             | Na <sub>2</sub> O <sub>2</sub> Bleach  |                                                 | Hunter Brightness of Pulp | Brightness Increment of Bleach |
|--------------------------------|---------------------|---------|-------------|-------------|----------------------------------------|-------------------------------------------------|---------------------------|--------------------------------|
| Acid used                      | Percent Consistency | Pulp pH | Time (min.) | Pulp Washed | Percent Na <sub>2</sub> O <sub>2</sub> | Percent Residual Na <sub>2</sub> O <sub>2</sub> |                           |                                |
| -----                          | -----               | -----   | -----       | -----       | 0.5                                    | 27.2                                            | 73.7                      | 5.1                            |
| H <sub>2</sub> SO <sub>4</sub> | 4                   | 6.05    | 15          | Yes         | 0.5                                    | 32.3                                            | 78.8                      | -----                          |
| H <sub>2</sub> SO <sub>4</sub> | 4                   | 6.05    | 15          | Yes         | 0.5                                    | 32.3                                            | 75.7                      | -----                          |
| H <sub>2</sub> SO <sub>4</sub> | 4                   | 5.05    | 15          | Yes         | 0.5                                    | 34.0                                            | 80.3                      | 6.6                            |
| H <sub>2</sub> SO <sub>4</sub> | 4                   | 5.05    | 15          | Yes         | 0.5                                    | 34.0                                            | 76.1                      | 7.8                            |
| H <sub>2</sub> SO <sub>4</sub> | 4                   | 4.10    | 15          | Yes         | 0.5                                    | 33.1                                            | 81.5                      | 7.8                            |
| H <sub>2</sub> SO <sub>4</sub> | 4                   | 4.10    | 15          | Yes         | 0.5                                    | 33.1                                            | 81.3                      | 7.8                            |

## EXAMPLE IV

Another set of experiments was conducted to study the effect of the acid treatment time. Table 4 shows the effects on kraft pulp B. The samples were subjected to the same calcium hypochlorite bleaching treatment. About 1.8% available chlorine was used at a bleach time

15 time was 1.5 hours. The final pH was 8.55 and the present residual chlorine was 20.8. Data is shown in Table 5 below. Pulp consistencies of 4 and 12% gave in the acid treatment stage substantially equal brightness increments. Thus, the pulp consistency in the acid treatment may vary over a relatively wide range.

Table 5

| Acid Treatment                 |                     |         |             |             | Na <sub>2</sub> O <sub>2</sub> Bleach  |                                                 | Hunter Brightness of Pulp | Brightness Increment of Bleach |
|--------------------------------|---------------------|---------|-------------|-------------|----------------------------------------|-------------------------------------------------|---------------------------|--------------------------------|
| Acid used                      | Percent Consistency | Pulp pH | Time (min.) | Pulp Washed | Percent Na <sub>2</sub> O <sub>2</sub> | Percent Residual Na <sub>2</sub> O <sub>2</sub> |                           |                                |
| -----                          | -----               | -----   | -----       | -----       | 0.35                                   | 3.6                                             | 76.3                      | 2.8                            |
| H <sub>2</sub> SO <sub>4</sub> | 4                   | 5.35    | 27          | Yes         | 0.35                                   | 9.7                                             | 79.1                      | -----                          |
| H <sub>2</sub> SO <sub>4</sub> | 4                   | 5.35    | 27          | Yes         | 0.35                                   | 9.7                                             | 78.8                      | -----                          |
| H <sub>2</sub> SO <sub>4</sub> | 12                  | 4.50    | 30          | Yes         | 0.35                                   | 9.7                                             | 82.6                      | 6.3                            |
| H <sub>2</sub> SO <sub>4</sub> | 12                  | 4.50    | 30          | Yes         | 0.35                                   | 9.7                                             | 79.6                      | -----                          |
|                                |                     |         |             |             |                                        |                                                 | 83.2                      | 6.9                            |

of 1.5 hours. The final pH was 8.5 and the residual 35 chlorine value was 14.0. Good brightness values are obtained with acid treatment times of from 5 up to 30 minutes. It should be noted that not much increase in brightness is noted when the time period is increased from 15 up to 30 minutes.

40

Table 4

| Acid Treatment                 |                     |         |             |             | Na <sub>2</sub> O <sub>2</sub> Bleach  |                                                 | Hunter Brightness of Pulp | Brightness Increment of Bleach |
|--------------------------------|---------------------|---------|-------------|-------------|----------------------------------------|-------------------------------------------------|---------------------------|--------------------------------|
| Acid used                      | Percent Consistency | Pulp pH | Time (min.) | Pulp Washed | Percent Na <sub>2</sub> O <sub>2</sub> | Percent Residual Na <sub>2</sub> O <sub>2</sub> |                           |                                |
| -----                          | -----               | -----   | -----       | -----       | 0.35                                   | 9.7                                             | 76.7                      | 2.8                            |
| H <sub>2</sub> SO <sub>4</sub> | 4                   | 5.15    | 5           | Yes         | 0.35                                   | 17.0                                            | 79.5                      | -----                          |
| H <sub>2</sub> SO <sub>4</sub> | 4                   | 5.15    | 5           | Yes         | 0.35                                   | 17.0                                            | 78.0                      | -----                          |
| H <sub>2</sub> SO <sub>4</sub> | 4                   | 5.10    | 15          | Yes         | 0.35                                   | 10.9                                            | 81.5                      | 4.8                            |
| H <sub>2</sub> SO <sub>4</sub> | 4                   | 5.10    | 15          | Yes         | 0.35                                   | 10.9                                            | 78.3                      | -----                          |
| H <sub>2</sub> SO <sub>4</sub> | 4                   | 5.20    | 30          | Yes         | 0.35                                   | 10.9                                            | 81.4                      | 4.7                            |
| H <sub>2</sub> SO <sub>4</sub> | 4                   | 5.20    | 30          | Yes         | 0.35                                   | 10.9                                            | 79.2                      | -----                          |
| H <sub>2</sub> SO <sub>4</sub> | 4                   | 5.20    | 30          | Yes         | 0.35                                   | 10.9                                            | 82.1                      | 5.4                            |

## EXAMPLE V

A study was also made of the effect of the consistency of the pulp when subjected to the acid treatment. Kraft pulp B was used for these tests. A calcium hypochlorite bleach stage preceded the acid treatment in every case. The percent available chlorine used was 1.8 and the bleach

time of 1.5 hours to give a final pulp pH of 8.5 and 20.2% residual chlorine. The results are shown in Table 6.

60 These data indicate that, of those tested, H<sub>2</sub>SO<sub>4</sub> and HCl are the preferred acids for the acid treatment. Sulfur dioxide appears to be somewhat less satisfactory, and alum is considered to be unsatisfactory.

Table 6

| Acid Treatment                                  |                     |         |             |             | Na <sub>2</sub> O <sub>2</sub> Bleach  |                                                 | Hunter Brightness of Pulp | Brightness Increment of Bleach |
|-------------------------------------------------|---------------------|---------|-------------|-------------|----------------------------------------|-------------------------------------------------|---------------------------|--------------------------------|
| Acid used                                       | Percent Consistency | Pulp pH | Time (min.) | Pulp Washed | Percent Na <sub>2</sub> O <sub>2</sub> | Percent Residual Na <sub>2</sub> O <sub>2</sub> |                           |                                |
| H <sub>2</sub> SO <sub>4</sub>                  | 4                   | 4.10    | 13          | Yes         | -----                                  | -----                                           | 78.0                      | -----                          |
| H <sub>2</sub> SO <sub>4</sub>                  | 4                   | 4.10    | 13          | Yes         | 0.35                                   | 7.3                                             | 78.5                      | -----                          |
| HCl                                             | 4                   | 4.05    | 15          | Yes         | 0.35                                   | 13.3                                            | 81.8                      | 3.8                            |
| HCl                                             | 4                   | 4.05    | 15          | Yes         | 0.35                                   | 13.3                                            | 78.6                      | -----                          |
| H <sub>2</sub> SO <sub>3</sub>                  | 4                   | 4.20    | 17          | Yes         | 0.35                                   | 20.6                                            | 82.0                      | 4.0                            |
| H <sub>2</sub> SO <sub>3</sub>                  | 4                   | 4.20    | 17          | Yes         | 0.35                                   | 20.6                                            | 77.8                      | -----                          |
| Al <sub>2</sub> (SO <sub>4</sub> ) <sub>3</sub> | 4                   | 5.1     | 16          | Yes         | 0.35                                   | 14.7                                            | 81.3                      | 3.3                            |
| Al <sub>2</sub> (SO <sub>4</sub> ) <sub>3</sub> | 4                   | 5.1     | 16          | Yes         | 0.35                                   | 14.7                                            | 74.8                      | -----                          |
|                                                 |                     |         |             |             |                                        |                                                 | 80.5                      | 2.5                            |

**9**  
**EXAMPLE VII**

A series of tests was also conducted on pulp Sample B to show that sodium hypochlorite could be used equally as well as calcium hypochlorite in the hypochlorite bleach stage. The percent available chlorine was 1.6 and the bleach time was 1.5 hours. A final pH of 9.2 and 23.7% residual chlorine was found. Data are tabulated in Table 7.

Table 7

| Acid Treatment                 |                     |         |             |             | Na <sub>2</sub> O <sub>2</sub> Bleach  |                                                 | Hunter Brightness of Pulp | Brightness Increment of Bleach |
|--------------------------------|---------------------|---------|-------------|-------------|----------------------------------------|-------------------------------------------------|---------------------------|--------------------------------|
| Acid used                      | Percent Consistency | Pulp pH | Time (min.) | Pulp Washed | Percent Na <sub>2</sub> O <sub>2</sub> | Percent Residual Na <sub>2</sub> O <sub>2</sub> |                           |                                |
| -----                          | -----               | -----   | -----       | -----       | 0.35                                   | 41.5                                            | 72.5                      | 4.1                            |
| H <sub>2</sub> SO <sub>4</sub> | 4                   | 5.05    | 15          | Yes         | 0.35                                   | 37.9                                            | 76.6                      | -----                          |
| H <sub>2</sub> SO <sub>4</sub> | 4                   | 5.05    | 15          | Yes         | 0.35                                   | 37.9                                            | 74.2                      | -----                          |
| HCl                            | 4                   | 5.2     | 15          | Yes         | 0.35                                   | 37.9                                            | 80.8                      | 8.3                            |
| HCl                            | 4                   | 5.2     | 15          | Yes         | 0.35                                   | 37.9                                            | 74.6                      | -----                          |
|                                |                     |         |             |             |                                        |                                                 | 80.9                      | 8.4                            |

## EXAMPLE VIII

The effect of washing the pulp before the acid treatment was also investigated. The tests shown were conducted on pulp B. In the hypochlorite bleach stage, 1.8% available chlorine was used and a bleach time of 1.5 hours. The results in brightness values are tabulated in Table 8. These data show that improved brightness values are obtained when the pulp is washed after the hypochlorite treatment and prior to the acid treatment. However, even better results are obtained when the pulp is directly acid treated following the hypochlorite stage with no intervening washing step. It is preferred to carry out the invention in this manner.

25 tration consisting of a 2% NaOH at 154° F. for about two hours. The washed pulp had a Hunter brightness of 30.1.

A portion of the alkaline extracted wood pulp was bleached with 2.5% available chlorine, as calcium hypochlorite, and 0.85% NaOH at 13% consistency and a 30 temperature of 96-99° F. for 1½ hours. The residual chlorine at this time was 28.1% or 0.702% available Cl<sub>2</sub> on dry pulp basis, and the pH was 9.8. For comparison purposes, one portion of the pulp indicated as Sample 35 E was directly treated with H<sub>2</sub>SO<sub>4</sub> at pH 5.0 and 4% consistency for 15 minutes according to the process of the invention. The remainder of the pulp batch was

Table 8

| Calcium Hypochlorite Bleach Stage |                   |             | Acid Treatment                 |                     |         |             | Na <sub>2</sub> O <sub>2</sub> Bleach  |                                               | Hunter Brightness of Pulp | Brightness Increment of Bleach |
|-----------------------------------|-------------------|-------------|--------------------------------|---------------------|---------|-------------|----------------------------------------|-----------------------------------------------|---------------------------|--------------------------------|
| Final pH                          | Residual Chlorine | Pulp Washed | Acid used                      | Percent Consistency | Pulp pH | Time (min.) | Percent Na <sub>2</sub> O <sub>2</sub> | Percent Resid. Na <sub>2</sub> O <sub>2</sub> |                           |                                |
| 8.55                              | 20.8              | -----       | -----                          | -----               | -----   | -----       | 0.35                                   | 3.6                                           | 76.3                      | -----                          |
| 8.55                              | 20.8              | Yes         | H <sub>2</sub> SO <sub>4</sub> | 4                   | 5.2     | 30          | 0.35                                   | 7.3                                           | 79.1                      | 2.8                            |
| 8.55                              | 20.8              | Yes         | H <sub>2</sub> SO <sub>4</sub> | 4                   | 5.2     | 30          | 0.35                                   | 7.3                                           | 76.9                      | -----                          |
| 8.55                              | 20.8              | No          | H <sub>2</sub> SO <sub>4</sub> | 4                   | 5.35    | 27          | 0.35                                   | 9.7                                           | 80.6                      | 4.3                            |
| 8.55                              | 20.8              | No          | H <sub>2</sub> SO <sub>4</sub> | 4                   | 5.35    | 27          | 0.35                                   | 9.7                                           | 78.8                      | -----                          |
|                                   |                   |             |                                |                     |         |             |                                        |                                               | 82.6                      | 6.3                            |

## EXAMPLE IX

To test the effect of pulp consistency during the peroxide bleaching treatment, an acid treated pulp sample was bleached at 4% consistency for three hours with the use of additional NaOH. Although a 4% consistency bleach generally gives only about one-half the response in brightness increment as does a high density bleach, the response in this bleaching step combined with acid treatment was outstanding. The overall brightness increment was 10.0, compared with a value of 10.3 on a 55 13% consistency bleach.

washed and centrifuged. One portion, Sample F, of this 55 washed pulp was adjusted to pH 5.0 by treatment with H<sub>2</sub>SO<sub>4</sub> at 4% consistency for 15 minutes. Another portion, Sample G, was treated with 0.702% available Cl<sub>2</sub> at pH 5.0 for 15 minutes. Both pulp Samples F and G were then washed and thickened. The remainder of the 60 washed pulp, Sample H, was evaluated for use as a control in measuring the brightness improvement obtained by the various treatment methods.

Table 9 below shows a résumé of the data on the preparation of the pulp. The percent residual chlorine

Table 9

| Bleached Pulp Sample | Percent Available Cl <sub>2</sub> | Pulp Washed after Hypochlorite Bleach | Percent H <sub>2</sub> SO <sub>4</sub> | Pulp pH | Percent Residual Chlorine | Hunter Brightness | Brightness Increment |
|----------------------|-----------------------------------|---------------------------------------|----------------------------------------|---------|---------------------------|-------------------|----------------------|
| H                    | 2.5                               | Yes                                   | None                                   | -----   | 128.1                     | 71.5              | -----                |
| E                    | -----                             | No                                    | 1.45                                   | 4.8     | 53.3                      | 76.5              | 5.0                  |
| F                    | -----                             | Yes                                   | 0.39                                   | 4.8     | -----                     | 73.1              | 1.6                  |
| G                    | 0.70                              | Yes                                   | 0.29                                   | 5.0     | 72.7                      | 75.4              | 3.9                  |

<sup>1</sup> Equivalent to 0.70% available Cl<sub>2</sub> on the dry pulp basis as used on Sample G.

values are based on the amount of residual chlorine at the end of the hypochlorite bleach.

The three acid treated pulps and the untreated pulp were then bleached with 0.5%  $\text{Na}_2\text{O}_2$ , 2% sodium silicate, and 0.10% NaOH at 13% consistency at 142° F. for two hours. The results are tabulated in Table 10 below.

Table 10

| Pulp used | Final Pulp pH | Percent Residual $\text{Na}_2\text{O}_2$ | Hunter Brightness | Brightness Increment |
|-----------|---------------|------------------------------------------|-------------------|----------------------|
| H         | 10.95         | 4.3                                      | 74.9              | 3.4                  |
| E         | 10.65         | 23.7                                     | 83.0              | 11.5                 |
| F         | 10.80         | 37.8                                     | 79.5              | 8.0                  |
| G         | 10.65         | 10.8                                     | 82.3              | 10.8                 |

These data indicate that the controlled acidification of the unwashed hypochlorite bleached pulp gives somewhat better brightness response than washing the pulp and giving an identical hypochlorous acid bleach with an equivalent amount of chlorine under the same conditions.

What is claimed is:

1. A process for producing a kraft pulp of improved brightness stability and strength which comprises chlorine bleaching a kraft pulp, alkali extracting said chlorine

bleached pulp, bleaching the resulting pulp with an alkaline hypochlorite bleach to provide a pulp of  $\text{pH } 9.5 \pm 1.0$  pH unit and containing a residual chlorine content of from 10 to 35% of the amount of the available chlorine from the alkaline hypochlorite, acidifying the resulting pulp containing said amount of residual chlorine with a non-reducing strong mineral acid to a pH of 4.0 to 5.5, and subjecting the resulting acidified pulp to at least one alkaline peroxide bleach to produce a pulp of improved strength and brightness stability.

5 2. A process, as defined in claim 1, wherein the non-reducing strong mineral acid is a member from the group consisting of sulfuric acid and hydrochloric acid.

## References Cited in the file of this patent

## UNITED STATES PATENTS

|           |         |               |
|-----------|---------|---------------|
| 1,768,821 | Bradley | July 1, 1930  |
| 1,771,064 | Rue     | July 22, 1930 |
| 1,820,502 | Schuber | Aug. 25, 1931 |
| 2,203,205 | Rawling | June 4, 1940  |
| 2,668,095 | Fennell | Feb. 2, 1954  |

## OTHER REFERENCES

25 Aitken: Peroxides to Bleach Sulphate Pulp, Canadian Chem. Processing, February 1953, pp. 42 and 44.